

# UNITED STATES PATENT OFFICE.

WILLIAM H. ALLEN, OF DETROIT, MICHIGAN.

## METAL-POLISH.

1,280,939.

Specification of Letters Patent.

Patented Oct. 8, 1918.

No Drawing.

Application filed December 7, 1917. Serial No. 205,945.

*To all whom it may concern:*

Be it known that I, WILLIAM H. ALLEN, a citizen of the United States, and residing at Detroit, in the county of Wayne and State of Michigan, have invented a new and Improved Metal-Polish, of which the following is a specification.

This invention relates to compositions for coating the surface of articles of iron or steel with carbon, preferably in the form of lamp-black or graphite, and its object is to provide a coating composition which will adhere to the metal surface, which may be rubbed or brushed to produce a polished surface, and which will prevent the metal surfaces coated thereby from rusting.

The metal polish may consist of one pound of finely divided graphite, three ounces of lamp-black and sufficient dilute phosphoric acid to make a thin paste. A seven per cent. solution of the acid or an equivalent solution of any salt of phosphoric acid having an acid reaction will usually be found satisfactory, although a stronger solution may be used. The proportions of graphite and

lamp-black may be varied if desired. This paste is applied to the surface of iron or steel, and when dry is rubbed or brushed. The phosphoric acid or the acid salts of phosphoric acid attack the iron or steel, forming phosphates of iron which adhere to the iron, and particles of the carbon intermingled with the phosphates are united to the metal by these phosphates. When dry, the surface may be rubbed with paraffin oil to brighten the finish.

I claim:

1. A metal polish consisting of finely divided graphite and lamp black and sufficient dilute phosphoric acid to form a thin paste. 40

2. A metal polish consisting of sixteen parts by weight of graphite, three parts by weight of lamp-black and sufficient dilute phosphoric acid to form a thin paste.

3. A metal polish consisting of finely divided graphite and lamp-black and sufficient dilute acid compound of phosphorus to form a thin paste. 45

WILLIAM H. ALLEN.